

## UNITED STATES PATENT OFFICE

CAMILLE DREYFUS, OF NEW YORK, N. Y., AND HERBERT PLATT, OF CUMBERLAND, MARYLAND, ASSIGNORS TO CELANESE CORPORATION OF AMERICA, A CORPORATION OF DELAWARE

## METHOD OF TREATING TEXTILE MATERIAL AND PRODUCT THEREOF

No Drawing.

Application filed July 30, 1929. Serial No. 382,274.

This invention relates to the treatment of textile material containing organic derivatives of cellulose whereby its lustre may be diminished.

10 An object of our invention is to treat textile materials containing organic derivatives of cellulose whereby their lustre may be reduced wholly or in part.

Other objects of our invention will appear 10 from the following detailed description.

In accordance with our invention we reduce the lustre of textile materials containing yarns of organic derivatives of cellulose by applying thereto a substance containing 15 an ethanolamine, and then subjecting the same to the action of a hot aqueous medium, such as steam under pressure or steam under atmospheric pressure superheated to 101° C. or more.

20 The textile material to be treated in accordance with our invention may be a woven or knitted fabric, or it may be in the form of yarn. The textile material may contain filaments of organic derivatives of cellulose

25 such as organic esters of cellulose and cellulose ethers. Examples of organic esters of cellulose are cellulose acetate, cellulose formate, cellulose propionate and cellulose butyrate, while examples of cellulose ethers 30 are ethyl cellulose, methyl cellulose and benzyl cellulose.

If desired, the textile material may be a mixed material containing yarns of organic derivatives of cellulose and yarns of other 35 fibres such as cotton, natural silk, reconstituted cellulose, wool, etc.

In order to reduce the lustre, a substance containing an ethanolamine is applied to the organic derivative of cellulose material.

40 While we have found that the best results are attained by employing triethanolamine, yet diethanolamine or monoethanolamine may be employed with advantage, particularly in admixture with the triethanolamine.

45 Preferably these materials are applied in the presence of some water.

If desired, the fabric or yarn of organic derivative of cellulose may have its lustre 50 reduced over the whole surface thereof by the

immersion of the same in an aqueous solution containing triethanolamine. For differential lustre effects, the substance containing the triethanolamine may be applied locally, either by brushing or spraying through stencils, or by printing in the form of a paste containing a suitable thickener such as starch, British gum, etc.

55 Yarn may be delustered by our process and the delustered yarn may be associated by 60 weaving with yarns of normal lustre, whereby fabrics having differential lustre effects may be produced. Thus if such yarns of different lustres are woven in a jacquard loom, a fabric having lustrous patterns 65 against delustered background or vice versa may be produced. By locally applying the substance containing triethanolamine to yarn, yarn of differential lustre may be produced, which may be woven into fabric having beau- 70

75 If a suitable dyestuff is added to the substance containing the triethanolamine, further enhanced effects may be obtained. For instance, if a paste containing the triethanolamine and the dyestuff is locally applied to the fabric, colored delustered patterns against a lustrous uncolored background are produced.

In the execution of our invention, we have 80 found that after the application of the substance containing the triethanolamine, the same should preferably be subjected to the hot steam without intermediate drying, since if the textile material is dried after the application of the triethanolamine and then steamed, the amount of delustering produced 85 is considerably diminished.

In order further to illustrate our invention 90 but without being limited thereto, the following specific examples are given.

## Example I

95 A fabric consisting wholly of yarns of cellulose acetate is padded with an aqueous solution containing 10% of triethanolamine. The fabric is then immediately subjected to the action of steam at 5 lbs. pressure for 15 min- 100

utes in a cottage steamer. The fabric is well delustered.

*Example II*

5 A fabric consisting wholly of cellulose acetate yarn is printed by means of engraved rollers having suitable designs with a paste made up as follows:

Corn starch thickener (1:1.5) 10 35 parts by weight  
British gum thickener (1:1) 15 parts by weight  
Triethanolamine 10 parts by weight

15 The fabric is immediately without drying, subjected to the action of steam at 10 lbs. pressure for 15 minutes in a cottage steamer. That part of the fabric to which the paste has been applied has its lustre very 20 much reduced, thus producing delustered patterns against lustrous background.

*Example III*

25 A fabric consisting wholly of cellulose acetate yarn has locally applied thereto the following paste:

Corn starch thickener (1:1.5) 35 parts by weight  
30 British gum thickener (1:1) 15 parts by weight  
Glycerine 5 parts by weight  
Triethanolamine 25 5 parts by weight

40 As an Example II, the fabric is immediately subjected to the action of steam at 10 lbs. pressure for 15 minutes, and delustered patterns against lustrous background are produced.

45 It is to be understood that the foregoing detailed description is given merely by way of illustration, and that many variations may be made therein, without departing from the spirit of our invention.

Having described our invention, what we claim and desire to secure by Letters Patent is:

50 1. Method of treating textile materials containing organic derivatives of cellulose comprising applying to at least part of the surface thereof a substance containing an ethanolamine, and then subjecting the material to the action of a hot aqueous medium.

55 2. Method of treating textile materials containing organic derivatives of cellulose comprising applying to at least part of the surface thereof a substance containing mono-ethanolamine, and then subjecting the material to the action of a hot aqueous medium.

60 3. Method of treating textile materials containing cellulose acetate comprising applying to at least part of the surface thereof a substance containing monoethanolamine, and then subjecting the material to the action of a hot aqueous medium.

then subjecting the material to the action of a hot aqueous medium.

4. Method of treating textile materials containing organic derivatives of cellulose comprising applying to at least part of the surface thereof a substance containing diethanolamine, and then subjecting the material to the action of a hot aqueous medium. 70

5. Method of treating textile materials containing cellulose acetate comprising applying to at least part of the surface thereof a substance containing diethanolamine, and then subjecting the material to the action of a hot aqueous medium. 75

6. Method of treating textile materials containing cellulose acetate comprising applying to at least part of the surface thereof a substance containing an ethanolamine, and then subjecting the material to the action of a hot aqueous medium. 80

7. Method of treating textile materials containing organic derivatives of cellulose comprising applying to at least part of the surface thereof a substance containing triethanolamine, and then subjecting the material to the action of a hot aqueous medium. 85

8. Method of treating textile materials containing cellulose acetate comprising applying to at least part of the surface thereof a substance containing triethanolamine, and then subjecting the material to the action of a hot aqueous medium. 90

9. Method of imparting a differential luster effect to fabric containing yarns of organic derivatives of cellulose comprising locally applying thereto a substance containing triethanolamine, and then subjecting the same to hot steam. 100

10. Method of imparting a differential luster effect to fabric containing yarns of cellulose acetate comprising locally applying thereto a substance containing triethanolamine, and then subjecting the same to hot steam. 105

11. Method of producing differential luster effects on fabrics containing yarns of cellulose acetate comprising locally printing the same with a paste containing triethanolamine, and then without intermediate drying subjecting the same to the action of hot steam. 110

12. Method of producing differential luster effects on fabric containing yarns of cellulose acetate comprising locally printing the same with a paste containing triethanolamine and glycerine, and then without intermediate drying subjecting the same to the action of hot steam. 115

13. Method of treating textile materials containing organic derivatives of cellulose comprising applying to at least part of the surface thereof a substance containing mono- and triethanolamine, and then subjecting the material to the action of a hot aqueous medium. 120

14. Method of treating textile materials 125

containing cellulose acetate comprising applying to at least part of the surface thereof a substance containing mono- and triethanolamine, and then subjecting the material to the action of a hot aqueous medium.

15. Method of treating textile materials containing organic derivatives of cellulose comprising applying to at least part of the surface thereof a substance containing di- and triethanolamine, and then subjecting the material to the action of a hot aqueous medium.

16. Method of treating textile materials containing cellulose acetate comprising applying to at least part of the surface thereof a substance containing di- and triethanolamine, and then subjecting the material to the action of a hot aqueous medium.

In testimony whereof, we have hereunto  
20 subscribed our names.

CAMILLE DREYFUS.  
HERBERT PLATT.

25

30

35

40

45

50

55

60